

# UNITED STATES PATENT OFFICE.

WILLIS R. WHITNEY, OF NISKAYUNA, NEW YORK, ASSIGNOR TO GENERAL ELECTRIC COMPANY, A CORPORATION OF NEW YORK.

## COATED STRAIN-HARDENED METAL.

1,331,888.

Specification of Letters Patent. Patented Feb. 24, 1920.

No Drawing.

Application filed June 15, 1918. Serial No. 240,177.

*To all whom it may concern:*

Be it known that I, WILLIS R. WHITNEY, a citizen of the United States, residing at Niskayuna, in the county of Schenectady, State of New York, have invented certain new and useful Improvements in Coated Strain-Hardened Metals, being a continuation in part of application Serial No. 192,129, filed September 19, 1917, of which

10 the following is a specification.

The brittleness produced in strain-hardened ferrous metals, particularly spring steel, caused by the action of an acid bath or by electrolysis has constituted a long-standing problem. It has been found to be impracticable, for example, to copper plate steel springs to decrease corrosion because the tensile strength of the springs was very greatly reduced by the plating. Pickling

15 steel springs in acid to clean the surface likewise greatly reduced the tensile strength. Experiments which have been made indicate that the deleterious effect is connected in some way with the generation of hydrogen

20 at the surface of the ferrous metal.

I have discovered that this deleterious effect may be obviated by providing metal under strain before being subjected to a hydrogen-generating bath, with a coating of

25 material which is substantially impervious to nascent hydrogen, for example, metallic tin. The metal thus coated may subsequently be electro-plated without any deleterious effects upon its mechanical properties.

30 In carrying out my invention which includes both a process and a new article resulting therefrom, the metal to be coated is preferably first cleaned mechanically, for

40 example, by sand blasting, and is then dipped, in the presence of a suitable flux, into a coating metal. When thus treating a metal such as spring steel which has been given a temper or set under strain, it is

45 necessary that a plating material should be chosen which has a melting point below the temperature at which the metal has been tempered. In case of spring steel the tempering temperature is somewhere about 300°

50 C. As tin has a melting point of 232°, and as it can readily adhere to a clean surface of ferrous metal, it is particularly well suited for the purpose of my invention. The cleaned steel springs or other strain-hardened articles to be coated, may be dipped

into the tin bath in the presence of rosin or other suitable flux. Subsequent to the tinning operation the steel articles may be electroplated in the usual way, for example, with copper, without impairing their mechanical properties.

60 The following specific figures will illustrate the benefits of my invention. Two steel springs were selected from a lot of springs, samples of which upon test had 65 broken on the testing machine with a pull varying between 310 and 439 pounds. The selected test springs were made cathode for one-half hour in a copper cyanid solution and when tested were found to break at 69 70 and 137 pounds pull respectively. The electrolytic treatment had reduced the breaking strength to about 22% and 31% respectively, of the average value of strength of similar untreated springs. Furthermore, the copper plated samples stretched very little before they broke, while the untreated stretched one or two times their original length. Two more test springs were pickled 75 respectively for three minutes and one hour 80 in a 20% sulfuric acid solution. The sample pickled for three minutes broke at 198 pounds showing a reduction of strength to 50% of the untreated value and the second sample pickled for one hour, broke at 29 85 pounds with a reduction in strength to 7% of the untreated value. The latter sample had been reduced by but one-thousandth of an inch in diameter by the action of the acid, which clearly shows that diminution of size 90 does not account for the weakening of the metal.

Additional samples of steel springs were first sand blasted, dipped into molten rosin and then into molten tin heated to a temperature of about 260 to 300° C. After having been tinned the samples were copper plated in the same solution used for copper plating the test samples above described. These tin plated samples showed a breaking 95 strength ranging from 318 to 417 pounds, all being well within the range of the tensile strength values obtained for the untreated springs. In other words, the mechanical properties of the samples had not been appreciably affected by the tin treatment and these properties were retained during a subsequent electrolytic treatment.

100 Although I have described the benefits of my invention with particular reference to 110

strained spring steel, I desire it to be understood that my invention is also applicable with beneficial result to other forms of strain-hardened steel, for example, steel articles of various sorts which have been formed by cold pressing or otherwise strained beyond their elastic limit.

What I claim as new and desire to secure by Letters Patent of the United States, is:—

- 10 1. The process of preventing ferrous metal while under strain from becoming brittle by the action of a hydrogen-generating agent which consists in providing said metal with a coating of material which is substantially impermeable to hydrogen, and then subjecting the metal to said agent.
- 15 2. The process of electroplating strain-hardened ferrous metal which consists in first providing said metal with a coating of conductive material such as tin impermeable to nascent hydrogen while preventing electrolytic action, and then subjecting to a desired electro-plating treatment.
- 20 3. The process of preventing strain-hardened steel from becoming brittle by the action of an electrolytic bath which consists in providing said steel with a coating of tin while preventing the generation of hydrogen at the surface of said steel, and then subjecting the coated steel to the desired electrolytic treatment.
- 25 4. The process of plating strain-hardened steel by electrolysis which consists in apply-

ing to said steel a coating of tin in the absence of an agent generating hydrogen, and then applying a desired metal by electrolysis.

5. The process of coating steel springs which consists in mechanically cleaning said springs, applying a coating of tin in the presence of a resinous flux and then applying a desired coating of metal by electrolysis.

6. An article of manufacture comprising ferrous spring metal, a coating of tin thereon and a coating of electro-deposited metal upon said tin, said metal having substantially the same mechanical properties as unplated metal of the same character.

7. An article of manufacture, comprising a steel spring, a coating of tin thereon, and a coating of electro-deposited copper upon said tin, said spring having substantially the same mechanical properties as unplated steel of the same character.

8. An article of manufacture, comprising a strain-hardened ferrous metal, a coating of conductive material substantially impermeable to hydrogen upon said steel, and a coating of electro-deposited metal upon said material, said metal having substantially the same mechanical properties as unplated metal of the same character.

In witness whereof, I have hereunto set my hand this 13th day of June, 1918.

WILLIS R. WHITNEY.